

P. C. SEEL,  
ANTISTATIC PHOTOGRAPHIC FILM,  
APPLICATION FILED DEC. 31, 1920.

1,434,454.

Patented Nov. 7, 1922.



WITNESS

*Harold A. Stewart.*

INVENTOR

*Paul C. Seel,*  
BY *R. L. Strainfield*

ATTORNEY

## UNITED STATES PATENT OFFICE.

PAUL C. SEEL, OF ROCHESTER, NEW YORK, ASSIGNOR TO EASTMAN KODAK COMPANY,  
OF ROCHESTER, NEW YORK, A CORPORATION OF NEW YORK.

## ANTISTATIC PHOTOGRAPHIC FILM.

Application filed December 31, 1920. Serial No. 434,354.

To all whom it may concern:

Be it known that I, PAUL C. SEEL, a citizen of the United States of America, residing at Rochester, in the county of Monroe 5 and State of New York, have invented certain new and useful Improvements in Anti-static Photographic Films, of which the following is a full, clear, and exact specification.

10 This invention relates to photographic film.

The principal object of my invention is to provide a photographic film having all of the usual qualities and possessing in addition 15 the property of preventing or greatly minimizing markings due to electrical discharges which are customarily referred to in the motion picture art as "static". Other objects will hereinafter appear.

20 I have found that photographic film may be rendered substantially anti-static by incorporating in the nitrocellulose base or support thereof certain substances together with small amounts of water. The preferred sub-

25 stances which I employ are glucose and glycerin. In place of the glucose analogous sugary substances may be employed and in place of the glycerin I may employ similar organic compounds of low volatility which 30 are hygroscopic or have a strong affinity for water and are substantially inert toward the photographic coatings.

In the accompanying drawing the single figure is a sectional view on an exaggerated 35 scale of a film embodying my invention.

In the drawing 1 is the base or support and 2 the sensitive layer.

In practice I mix the anti-static ingredients together and then add such mixture to 40 any of the usual nitrocellulose film dopes. In the preferred embodiment of my invention I add an amount of glucose equal to from 2 to 4% of the weight of the nitrocellulose in the dope, an amount of glycerin equal 45 to from 2 to 4% of the weight of the nitrocellulose in the dope and an amount of water equal to from 2 to 4% of the weight of the nitrocellulose in the dope. Of course, these proportions are merely illustrative and may 50 be varied considerably according to the thickness of the dope and the methods of spreading and curing the latter. But the preferred proportions herein described oper-

ate well under the standard film-making conditions.

As an illustration of the formula to which my anti-static mixture may be added the following is noted: 100 parts of nitrocellulose, 200 to 400 (say 250) parts of acetone, 200 to 400 (say 250) parts of methyl alcohol, 20 to 200 (say 40) parts of fusel oil. To this may be added, if desired, 1 to 30 (say 10) parts of camphor. My mixture of 4 parts of glucose, 4 parts of glycerin and 4 parts of water is then incorporated thorough- 65 ly in the dope.

The ingredients are those commonly used in the art, of sufficient purity to yield films of the desired transparency and relative freedom from color. Various volatile solvents may be used and either acetone or methyl alcohol can be used alone in a suitable amount or varying mixtures can be employed. For the fusel oil may be substituted the other monohydroxy aliphatic alcohols of 70 from 4 to 5 carbon atoms, like normal butyl and isobutyl alcohols.

The dope is spread and cured by the evaporation of the volatile solvents, so as to form a transparent flexible sheet or film 80 base in the usual way. On this support the sensitive photographic coatings or emulsions are applied and from the product motion picture films and other films are prepared as is well understood in the art. Such films 85 are notably resistant to defects from the electrical discharges. While I am inclined to attribute this property to the increased electrical conductivity of the film base, due to the moisture which is trapped or held there- 90 in by the glucose and glycerin, a knowledge of the theoretical basis of my invention is not necessary to the practicing of it, as hereinabove described. It should be noted that 95 the water, when incorporated with the substances and in the manner set forth in the examples given above, does not segregate in the film so as to impair the transparency of the latter.

The film base and dope are covered in my 100 co-pending divisional application, Serial No. 461,916, filed Apr. 16, 1921.

Having thus described my invention, what I claim as new and desire to secure by 105 Letters Patent is:

1. A photographic film comprising a

- sensitive coating on a nitrocellulose support which contains a sugar, an inert hygroscopic organic compound of low volatility and water.
5. 2. A photographic film comprising a sensitive coating on a nitrocellulose support which contains a sugar glycerin, and water.
3. A photographic film comprising a sensitive coating on a nitrocellulose support which contains glucose, an inert hygroscopic organic compound of low volatility and water.
4. A photographic film comprising a sensitive coating on a nitrocellulose support which contains glucose, glycerin and water.
5. A photographic film comprising a sensitive coating on a nitrocellulose support which contains an amount of a sugar equal to approximately 4% or less of the weight 20 of the nitrocellulose, an amount of an inert hygroscopic organic compound of low volatility equal to substantially 4% or less of the weight of the nitrocellulose and an amount of water equal to substantially 4% or less of the weight of the nitrocellulose.
6. A photographic film comprising a sensitive coating on a nitrocellulose support which contains an amount of a sugar equal to approximately 4% or less of the weight 30 of the nitrocellulose, an amount of glycerin equal to substantially 4% or less of the weight of the nitrocellulose and an amount of water equal to substantially 4% or less of the weight of the nitrocellulose.
7. A photographic film comprising a sensitive coating on a nitrocellulose support which contains an amount of glucose equal to substantially 4% or less of the weight of the nitrocellulose, an amount of an inert hygroscopic organic compound of low volatility equal to substantially 4% or less of the weight of the nitrocellulose and an amount of water equal to substantially 4% or less of the weight of the nitrocellulose.
8. A photographic film comprising a sensitive coating on a nitrocellulose support which contains an amount of glucose equal to substantially 4% or less of the weight of the nitrocellulose, an amount of glycerin equal to substantially 4% or less of the weight of the nitrocellulose and an amount of water equal to substantially 4% or less of the weight of the nitrocellulose.
9. A photographic film comprising a sensitive coating on a nitrocellulose support, which contains water and organic material for retaining and preventing precipitation of said water.

Signed at Rochester, New York, this 24th day of December, 1920.

PAUL C. SEEL.